

# UNITED STATES PATENT OFFICE.

HERMANN ENDEMANN, OF BROOKLYN, ASSIGNOR TO GUSTAV L. JAEGER,  
OF NEW YORK, N. Y.

## MANUFACTURE OF MATCHES.

SPECIFICATION forming part of Letters Patent No. 275,617, dated April 10, 1883.

Application filed January 24, 1883. (No specimens.)

*To all whom it may concern:*

Be it known that I, HERMANN ENDEMANN, a citizen of the United States, residing at Brooklyn, in the county of Kings and State of New York, have invented new and useful Improvements in the Manufacture of Matches, of which the following is a specification.

This invention consists in the combination, with a strip, stick, or sheet of paper, pasteboard, or wood saturated with oleic acid and with a suitable lighting composition, of basic binding material—such as protoxide of lead—which may be incorporated into the lighting composition or applied to the surface of the stock after the same has been treated with oleic acid.

My invention is intended particularly for matches where the lighting composition does not inclose the match, but is applied to a flat surface, as in a tape match or in a regular stick match, where the lighting composition is applied only at the end. In the manufacture of such matches, sticks or strips of paper, straw-board, or wood-board have heretofore been used, and the lighting composition has been applied to said sticks, strips, or sheets after the same were saturated with oleic acid. It is found, however, that the lighting composition applied to such sticks, strips, or sheets is liable to break off, since the materials generally used for the various lighting compositions have no affinity for the oleic acid used for saturating the stock—that is to say, the paper, pasteboard, or wood, or other material employed for the manufacture of matches.

After various experiments I have found that different substances of a basic character can be used as binding materials—such, for instance, as protoxide of lead, (litharge,) oxide of zinc, or oxide of magnesium. The binding material which I use by preference is litharge, and I have applied the same either by incor-

porating it with the lighting composition or by applying it to the saturated stock.

The lighting composition which I use by preference consists of phosphorus, three parts; fine sharp sand or powdered glass, two parts; gum-tragacanth, one-half part; water, three parts. If the basic binding material is to be incorporated with the lighting composition, I add to the mass above stated two parts of litharge or an equivalent quantity of oxide of zinc or other similar material. After the ingredients have been thoroughly mixed, so as to form a homogeneous mass, I bring the mass upon the saturated sticks or strips; or the stock may be saturated in sheets with oleic acid and the lighting composition applied thereto in rows at suitable distance apart, and after the rows have dried the sheet may be cut up in strips or sticks, which are finally packed for use. If I desire to apply the litharge or other basic binding material directly to the stock, I mix the same with a small quantity of a suitable gum and apply the mixture to the surface of the saturated stock before the lighting composition is applied.

What I claim as new, and desire to secure by Letters Patent, is—

In the manufacture of matches, the combination, with a stick, strip, or sheet of paper, pasteboard, or wood saturated with oleic acid and with a suitable lighting composition, substantially such as herein named, of a basic binding material—such as protoxide of lead—substantially in the manner and for the purpose set forth.

In testimony whereof I have hereunto set my hand and seal in the presence of two subscribing witnesses.

H. ENDEMANN. [L. S.]

Witnesses:

W. HAUFF,  
E. F. KASTENHUBER.